# EUROPEAN PATENT SPECIFICATION

(11) **EP 3 222 702 B1**
(45) Date of publication and mention of the grant of the patent: **05.01.2022**
(21) Application number: 15861457.8
(22) Date of filing: 18.11.2015
(51) Int. Cl.: C10M 169/04, C10N 10/04, C10N 20/00, C10N 20/02, C10N 20/04, C10N 30/00, C10N 40/25

(54) **CYLINDER LUBRICATING OIL COMPOSITION FOR SCRUBBER-EQUIPPED CROSSHEAD DIESEL ENGINES**
ZYLINDER SCHMIERÖLZUSAMMENSETZUNG FÜR MIT SCHRUBBER AUSGESTATTETE KREUZKOPFDIESELMOTOREN
COMPOSITION D'HUILE DE LUBRIFICATION DE CYLINDRES POUR MOTEURS DIESEL À CROSSE ÉQUIPÉS D'UN ÉPURATEUR

(30) Priority: 18.11.2014 JP 2014234045; 18.11.2014 JP 2014234046
(43) Date of publication of application: 27.09.2017
(73) Proprietor: JXTG Nippon Oil & Energy Corporation, Chiyoda-ku Tokyo 1008162 (JP)
(72) Inventor: TAKESHIMA, Shigeki, Tokyo 100-8162 (JP)
(74) Representative: Hoffmann Eitle
(86) International application number: PCT/JP2015/082411
(87) International publication number: WO 2016/080441

(56) References cited:
- WO-A1-99/64543
- WO-A1-2014/172125
- JP-A- 2005 002 341
- JP-A- 2009 185 293
- JP-A- 2010 174 092
- JP-A- 2011 132 338
- JP-A- 2011 157 960
- US-A1- 2012 258 897
- TAKESHIMA , S: 'Influence of Countermeasure Technologies for SOx Regulation on Engine Lubrication' JOURNAL OF THE JAPAN INSTITUTE OF MARINE ENGINEERING vol. 50, no. 3, 01 January 2015, pages 72 - 78, XP055445521

## Description

### TECHNICAL FIELD

The present invention relates to a cylinder lubricating oil composition for a crosshead diesel engine equipped with a scrubber, and specifically relates to a cylinder lubricating oil composition suitable for use in a crosshead diesel engine equipped with a scrubber.

### BACKGROUND

Crosshead diesel engines are used a lot for main engines of large ships. Thus, it can be said that large part of the effect of ship operations on the environment is from emission matter of crosshead diesel engines.

Interests in environmental problems have been increased, and attentions are also given to nitrogen oxides (NOx) and sulfur oxides (SOx) contained in exhaust gases emitted from ships to the air. Regarding NOₓ regulations, International Maritime Organization (IMO) decided to put Tier III into effect in Emission Control Area from 2016. Regarding SOₓ regulations, discussed is to reduce the sulfur components in fuels used in General Sea Area into no more than 0.5 %, from 2020 or 2025.

As a technique to reduce the concentrations of SOₓ and NOₓ in exhausted gases from ships, applications of scrubber techniques are focused on. As a NOₓ reduction technique conforming to IMO Tier III, EGR (Exhaust Gas Recirculation) scrubbers (Patent Literatures 1 to 4) are focused on. As options to reduce SOₓ emission amount, considered are to reduce the sulfur components in fuels (use of low-sulfur fuels), and to make the amounts of sulfur oxide emitted from conventional high-sulfur fuels same as the amounts of sulfur oxide emitted from low-sulfur fuels of no more than 0.5 % in sulfur component, by means of exhaust gas aftertreatment apparatuses. The latter option is more focused on because low-sulfur fuels are expensive. There is a suggestion of a de-SOₓ treatment by means of a scrubber as an exhaust gas aftertreatment apparatus (Patent Literature 5).

A scrubber (scrubbing dust collector) generally means a device to separate harmful substances (e.g. harmful gases and dusts) in exhaust gases, by collecting the harmful substances into liquid drops and liquid films of absorption liquids (e.g. water). For example, separation of SOₓ by absorbing it into an aqueous solution such as sodium hydroxide aqueous solution and separation of soot by density difference after the soot is collected in water phase are considered.

In order to efficiently collect harmful substances by scrubber, the gases and the absorption liquid need to sufficiently contact with each other. Thus, scrubbers are well made to increase the efficiency of gas-liquid mixing. However, exhaust gases from diesel engines include hydrocarbon-based substances such as unburnt fuel and lubricant mist. Such hydrocarbon-based substances do not dissolve in water, and may emulsify by strong mixing with water. If these hydrocarbon-substances and water are emulsified, the soot component in the exhaust gases are wrapped inside the emulsion to form scums, and the scums accumulate at the upper portion of the absorption liquid, as a result, the separation becomes difficult.

Patent Literature 6 discloses a method of lubricating a cylinder liner (and piston) of a 2-stroke internal combustion engine with a power output of at least 1600 kilowatts comprising supplying to the engine a lubricating composition comprising: an oil of lubricating viscosity; 3 wt % to 30 wt % of an alkaline earth or alkali metal sulphonate detergent; and an oil-soluble polyalkylene glycol having a distribution of molecular weight such that the molecules thereof have a weight of 2500 to less than 10,000 Daltons and comprise 0.05 wt % to 3 wt % of the lubricating composition.

Patent Literature 7 discloses a cylinder lubricant composition, for crosshead diesel engines, which contains alkaline earth metal phenate (0.005 mol/kg or more by phenate soap content), amine antioxidant (0.1-5 %mass) and oil-soluble molybdenum compound (30-500 mass ppm), in a base oil having aromatic content of 8.5 %mass or more. The composition has base number of 20-100 mg potassium hydroxide/g and a viscosity of 12.6 mm <2>/s or more at 100° C.

Patent Literature 8 discloses a diesel cylinder oil, having a viscosity of 15 to 27cS, a viscosity index of at least 95 and a total base number of at least 40 mg KOH/g, which comprises a neutral base stock of no more than 725 SUS viscosity (100 C), and from 2 to 15 wt. % of the oil of a oil soluble, liquid polyisobutylene having a viscosity from 1,500 to 8,000 cS (100 C).

Among engine oils used for diesel engines, system oils for crosshead diesel engines and engine oils for four-cycle trunk piston diesel engines are purified by centrifugal purifiers and repeatedly used for lubrication. In order to keep the cleaning effect by centrifugal purifier, water separation property is required of these lubricating oils. Cylinder oils for crosshead diesel engines are once-through type lubricating oils, that is, they are not cleaned by centrifugal purifiers or repeatedly used, and do not contact with water in centrifugal purifiers. Therefore, water separation property was not previously required of cylinder oils for crosshead diesel engines.

### Citation List

### Patent Literature

Patent Literature 1: JP 2011-157959 A
Patent Literature 2: JP 2011-157960 A
Patent Literature 3: JP 2012-137092 A
Patent Literature 4: JP H8-511074 T
Patent Literature 5: JP 2011-185275 A
Patent Literature 6: WO 2014/172125
Patent Literature 7: US2012/258897
Patent Literature 8: WO 99/64543

### Summary of Invention

### Technical Problem

An object of the present invention is to provide a cylinder lubricating oil composition for a crosshead diesel engine equipped with a scrubber, by which it is possible to improve water separation property and to reduce or inhibit generation of scums from hydrocarbon-based substances, soots and moisture in the scrubber.

### Solution to Problem

A first aspect of the present invention is a cylinder lubricating oil composition for a crosshead diesel engine equipped with a scrubber, as disclosed in the claims.

In the present description, "crosshead diesel engine equipped with a scrubber" means a crosshead diesel engine provided with a structure of purifying gases emitted from cylinders by at least one scrubber. The scrubber may be an EGR scrubber with which the gases that passed through the scrubber are guided to the inlet side of the cylinders (for example see Patent Literatures 1 to 4), and may be an exhaust gas scrubber with which the gases that passed through the scrubber are not guided to the inlet side of the cylinders (for example see Patent Literature 5). "Crosshead diesel engine" is typically a two-stroke crosshead diesel engine.

The first embodiment of the first aspect of the present invention is a cylinder lubricating oil composition for a crosshead diesel engine equipped with a scrubber, including:
a base oil;
(A) a metallic detergent; and
(B) a demulsifier in an amount of 0.02 to 5.0 mass% on the basis of the total mass of the composition, wherein the component (B) is one or more polyether compound;
   wherein the lubricating oil composition has a base number measured by perchloric acid method of of 15 to 125 mgKOH/g, and a kinematic viscosity at 100°C of 10 to 30 mm2/s
   and wherein the composition optionally comprises
(C) a nitrogen-containing ashless dispersant in an amount of no more than 0.2 mass% in terms of nitrogen on the basis of the total mass of the composition

The component (B) is one or more polyether compound. In such a configuration, it is preferable that the number average molecular weight of the component (B) is no less than 500. It is noted that, in the present invention, "polyether compound" means a compound having a polyether part, and the polyether part may be further modified by an ester bond and the like for example.

As a preferable embodiment of the first embodiment, a configuration in which the component (A) is a Ca phenate may be given for example.

The second embodiment of the first aspect of the present invention is a cylinder lubricating oil composition for a crosshead diesel engine equipped with a scrubber, including:
a base oil;
(A) a metallic detergent,
   wherein the lubricating oil composition comprises, as the component (A),
      (A1) a Ca phenate detergent; and
      (A2) a metallic detergent other than any Ca phenate detergent,
   wherein
      the lubricating oil composition optionally includes:
         (C-1) a succinimide having at least one alkyl or alkenyl group in a molecule thereof, or a borated derivative thereof, in an amount of no more than 0.015 mass% in terms of nitrogen on the basis of the total mass of the composition,
      the lubricating oil composition has a base number measured by perchloric acid method of of 15 to 125 mgKOH/g, and a kinematic viscosity at 100°C of 10 to 30 mm²/s,
         and
      the Ph value represented by the following formula (1) is no more than 20 × 10⁻³:$Ph value = {C}_{Ca} \times 2 / \left({r}_{M}\times 40.08\right)$ in the formula (1), C_{Ca} represents calcium content (mass%) derived from the component (A1), and r_{M} represents a metal ratio of the component (A1),
   wherein the metal ratio of component (A1) is calculated by formula (2): $\begin{matrix}metal ratio \left(A1\right) = calcium content in mass % in Ca phenate detergent which is component \left(A1\right) / calcium \\ content in mass % derived from soap base in Ca phenate detergent which is component \left(A1\right) .\end{matrix}$

As a preferable embodiment of the second embodiment, a configuration in which the lubricating oil composition includes the component (C) in an amount of greater than 0 mass% and no more than 0.015 mass% in terms of nitrogen on the basis of the total mass of the composition may be given for example.

As a preferable embodiment of the second embodiment, a configuration in which the component (A2) is a Ca sulfonate and/or a Ca salicylate may be given for example.

A second aspect of the present invention is a method of lubricating a cylinder of a crosshead diesel engine equipped with a scrubber, including:
operating the crosshead diesel engine while supplying the lubricating oil composition according to the first aspect of the present invention to the cylinder of the crosshead diesel engine equipped with the scrubber; and
purifying at least a part of gas exhausted from the cylinder in the scrubber.

In the second aspect of the present invention, the purifying in the scrubber may include contacting the gas introduced into the scrubber with water and/or a basic aqueous solution.

### Advantageous Effects of Invention

According to the first aspect of the present invention, it is possible to provide a cylinder oil for a crosshead diesel engine equipped with a scrubber, by which it is possible to reduce or inhibit generation of scums from hydrocarbon-based substances, soots and moisture in the scrubber.

According to the method of lubricating a cylinder of a crosshead diesel engine equipped with a scrubber of the second aspect of the present invention, it is possible to reduce or inhibit generation of scums from hydrocarbon-based substances, soots and moisture in the scrubber, in purification of gases emitted from the cylinder in the scrubber.

### DESCRIPTION OF EMBODIMENTS

Hereinafter, the present invention will be described in detail. It should be noted that, unless otherwise mentioned, "A to B" regarding numerical values A and B means "A or more and B or less". When the unit of the numerical value A is omitted, the unit given to the numerical value B is applied as the unit of the numerical value A.

### <Lubricating Base Oil>

As the base oil in the present invention, at least one selected from the group consisting of mineral oils and synthetic oils may be used.

The mineral oil is not particularly limited. General examples of the mineral oil include: a product made by fractional distillation of an atmospheric residue obtained by atmospheric distillation of a crude oil, by carrying out desulfuration and hydrogenolysis to have a desirable viscosity grade; and a product made by solvent dewaxing or contact dewaxing of the above-described atmospheric residue, on which a solvent extraction and hydrogenation are further carried out if necessary.

Further, as the mineral oil: an isomerized petroleum wax lubricating base oil made by hydroisomerizing a petroleum wax, which is a by-product in a dewaxing process in producing a base oil produced by carrying out a fraction distillation on an atmospheric distillation residual under reduced pressure to have a desirable viscosity grade, thereafter carrying out processes of solvent refining, hydrorefining, and the like, thereafter carrying out a solvent dewaxing; and an isomerized GTL wax lubricating base oil produced by a method of isomerizing GTL WAX (Gas To Liquid Wax) produced by a method of fisher-tropsh process may also be used. The basic production process of these isomerized wax lubricating base oils are the same as the production process of a hydrogenolysis base oil.

As the synthetic oil, synthetic oils used as general lubricating base oils may be used without particular limitations. Specific examples include: polybutenes and hydrides thereof; oligomers such as 1-octene, 1-decene and dodecene, and poly α-olefines and hydrides thereof which are oligomers and the like of mixtures of the above-mentioned oligomers; diesters such as ditridecyl glutarate, di-2-ethylhexyl adipate, diisodecyl adipate, ditridecyl adipate, di-2-ethylhexyl sebacate; polyolesters such as trimethylolpropane caprylate, trimethylolpropane pelargonate, pentaerythrytol-2-ethylhexanoate, pentaerythritol pelargonate; copolymers of dicarboxylic acids such as dibutyl maleate and C₂ to C₃₀ α-olefines; aromatic-based synthetic oils such as alkylnaphthalene, alkylbenzene, and aromatic esters; and mixtures thereof.

The kinematic viscosity at 100°C of the base oil is preferably no less than 10 mm²/s, more preferably no less than 14 mm²/s, and preferably no more than 25 mm²/s and more preferably no more than 20 mm²/s. By having such lower limit values or more of the kinematic viscosity at 100°C of the base oil, sufficient oil films may be formed at the lubricating points, and good lubricity may be obtained. By having such upper limit values or less of the kinematic viscosity at 100°C of the base oil, good fluidity at a low temperature may be obtained. In the present invention, the kinematic viscosity at 100°C means a kinematic viscosity at 100°C defined in ASTM D-445.

Examples of a preferable embodiment of the base oil include a mixture base oil of a base oil having a kinematic viscosity at 100°C of 10 to 14 mm²/s and a base oil having a kinematic viscosity at 100°C of 20 to 40 mm²/s.

The viscosity index of the base oil is preferably no less than 85, more preferably no less than 90, and especially preferably no less than 95. By having such lower limit values or more of the viscosity index of the base oil, the viscosity at a low temperature may be held down, and good startability may be obtained. In the present invention, the viscosity index means a viscosity index measured in conformity with JISK2283-1993.

The content of saturated component of the base oil based on the total amount of the base oil is preferably no less than 50 mass%, more preferably no less than 55 mass%, and preferably no more than 90 mass% and more preferably no more than 75 mass%. By having such lower limit values or more of the saturated component, good oxidation stability may be obtained. By having such upper limit values or less of the saturated component, sufficient solubility of asphaltene and deteriorated substances may be obtained, whereby good cleanliness is obtained. In the present description, the saturated component means a saturated component measured by the method described in ASTM D 2007-93.

### <(A) Metallic Detergent (1)>

In the first embodiment of the lubricating oil composition of the present invention, (A) metallic detergent (hereinafter referred to as "component (A)") is a so-called metallic detergent generally used in lubricating oils. Examples of the component (A) include phenate detergents, sulfonate detergents, and salicylate detergents. These metallic detergents may be used alone or in combination.

As the component (A), phenate detergents may be especially preferably used. Preferable examples of the phenate detergents include alkaline earth metal salts of compounds having a structure represented by the following formula (1), basic salts thereof, and overbased salts thereof. Examples of the alkaline earth metal salts include magnesium, barium, and calcium. Among them, magnesium and calcium are preferable, and calcium is especially preferable. The component (A) may be used alone or in combination.

In the formula (1), R¹ is a linear or branched, saturated or unsaturated C₆-C₂₁ alkyl or alkenyl group, m is a polymerization degree shown by an integer of 1 to 10, A is a sulfide (-S-) group or methylene (-CH₂-) group, x is an integer of 1 to 3. R¹ may be a combination of two or more different groups.

The carbon number of R¹ in the formula (1) is preferably 9 to 18, and more preferably 9 to 15. If the carbon number of R¹ is less than 6, the solubility to the base oil may degrade. If the carbon number of R¹ is more than 21, manufacturing is difficult, and the heat resistance may degrade.

The polymerization degree m in the formula (1) is preferably 1 to 4. By having the polymerization degree m within this range, the heat resistance may be improved.

The base number of the phenate detergent is preferably no less than 60 mg KOH/g, and more preferably no less than 100 mg KOH/g, and preferably no more than 350 mg KOH/g, and more preferably no more than 300 mg KOH/g. By having such lower limit values or more of the base number, good acid neutralizing property may be obtained, and by having such upper limit values or less of the base number, good detergent property may be obtained. In the present invention, the base number is measured by perchloric acid method.

Preferable examples of the sulfonate detergent include alkaline earth metal salts of alkyl aromatic sulfonc acids obtained by sulfonation of alkyl aromatic compounds, basic salts thereof, and overbased salts thereof. The weight average molecular weight of the alkyl aromatic compound is preferably 400 to 1500, and more preferably 700 to 1300. Examples of alkaline earth metal include magnesium, barium, and calcium. Magnesium and calcium are preferable, and calcium is especially preferable. Examples of the alkyl aromatic sulfonic acid include a so-called petroleum sulfonic acid and synthetic sulfonic acid. As the petroleum sulfonic acid mentioned here, a sulfonated alkyl aromatic compound of lubricating oil distillate of a mineral oil, and a so-called mahogany acid which is a by-product of white oil manufacturing may be given for example. As an example of the synthetic sulfonic acid, sulfonated alkylbenzene having a linear or brunched alkyl group, obtained by recovery of by-product in alkylbenzene manufacturing plant, the alkylbenzene being a raw material of cleansers, or by alkylation of benzene with polyolefin, may be given. As another example of the synthetic sulfonic acid, sulfonated alkylnaphthalenes such as sulfonated dinonylnaphthalene may be given. The sulfonating agent used in sulfonation of these alkyl aromatic compounds is not particularly limited, and fuming sulfuric acid and anhydrous sulfate may be used for example.

The base number of the sulfonate detergent is preferably no less than 10 mgKOH/g, more preferably no less than 150 mgKOH/g, and more preferably no less than 250 mgKOH/g, and preferably no more than 500 mgKOH/g, and more preferably no more than 450 mgKOH/g. By having such lower limit values or more of the base number, good acid neutralizing property may be obtained. By having such upper limit values or less of the base number, good detergent property may be obtained.

Preferable examples of the salicylate detergent include metal salicylates, basic salts thereof, and overbased salts thereof. As the metal salicylate mentioned herein, a compound represented by the following formula (2) may be given for example.

In the above formula (2), R² independently is a C₁₄-C₃₀ alkyl or alkenyl group, M is an alkaline earth metal, and n is 1 or 2. M is preferably calcium or magnesium, and especially preferably calcium. Preferably, n is 1. When n = 2, R² may be a combination of different groups.

Examples of a preferable embodiment of the salicylate detergent include an alkaline earth metal salicylate represented by the above formula (2) wherein n = 1, basic salt thereof, and overbased salt thereof.

The method for manufacturing the alkaline earth metal salicylate is not particularly limited, and a known method for manufacturing a mono alkyl salicylate may be employed. For example, the alkaline earth metal salicylate may be obtained by reacting monoalkyl salicylic acid and the like with metal base such as oxides and hydroxides of alkaline earth metals, or by once changing the monoalkyl salicylic acid and the like to be alkaline metal salts such as sodium salts and potassium salts, then metal-exchanging them with alkaline earth metal salts. The monoalkyl salicylic acid and the like are obtained from phenol as a starting raw material, by carrying out an alkylation on the phenol with olefin thereafter carrying out a carboxylation with carbon dioxide, or from salicylic acid as a starting raw material, by carrying out an alkylation on the salicylic acid with the olefin.

The method for obtaining a basic salt of the alkaline earth metal salicylate is not particularly limited. For example, the basic salt may be obtained by heating the alkaline earth metal salicylate and excess alkaline earth metal salt or excess alkaline earth metal basic salt (hydroxide or oxide of alkaline earth metal) in presence of water. The method for obtaining an overbased salt of the alkaline earth metal salicylate is not particularly limited. For example, the overbased salt may be obtained by reaction of the alkaline earth metal salicylate and the base of the hydroxide of the alkaline earth metal and the like, in presence of carbon dioxide, boric acid, or borate salt.

### AMENDMENTS FOR PROSECUTION IN THE EPO REGIONAL PHASE

The base number of the salicylate detergent is preferably no less than 60 mgKOH/g, more preferably no less than 100 mgKOH/g, and preferably no more than 350 mgKOH/g, and more preferably no more than 300 mgKOH/g. By having such lower limit values or more of the base number, good acid neutralizing property may be obtained. By having such upper limit values or less of the base number, good detergency may be obtained.

The metal ratio of the component (A) is preferably no less than 1, more preferably no less than 3, and preferably no more than 50 and more preferably no more than 30.

In the first embodiment of the lubricating oil composition of the present invention, as the component (A), one or more calcium detergent selected from the group consisting of Ca phenate detergents, Ca sulfonate detergents, and Ca salicylate detergents may be preferably used.

The Ca phenate detergents are the above-described phenate detergents in which calcium is used as the alkaline earth metal. That is, the Ca phenate detergent means a calcium salt, basic salt, or overbased salt of alkylphenol sulfide.

The Ca sulfonate detergents are the above-described detergents in which calcium is used as the alkaline earth metal. That is, the Ca sulfonate detergent means a calcium salt, basic salt, or overbased salt of an alkyl aromatic sulfonic acid.

The Ca salicylate detergents are the above-described salicylate detergents in which calcium is used as the metal. That is, the Ca salicylate detergent means calcium salicylate, or, a basic salt or overbased salt thereof. When a calcium detergent is used as the component (A), the content thereof is preferably 0.50 to 4.3 mass% in terms of calcium on the basis of the total mass of the lubricating oil composition.

### <(A) Metallic Detergent (2)>

The second embodiment of the lubricating oil composition of the present invention includes, as the component (A), (A1) a Ca phenate detergent and (A2) a metallic detergent other than any Ca phenate detergent.

### ((A1) Ca phenate detergent)

As (A1) Ca phenate detergent (hereinafter referred to as "component (A1)"), a calcium salt, basic salt, or overbased salt of a compound having a structure represented by the above formula (1) may be given. For the component (A1), one kind may be used alone, or two or more kinds may also be used in combination. A preferable embodiment of the component (A1) is as described above regarding the phenate detergent.
((A2) Metallic detergent other than any Ca phenate detergent)
(A2) Metallic detergent other than any Ca phenate detergent (hereinafter referred to as "component (A2)") is preferably a metallic detergent other than any phenate detergent. Examples of such a metallic detergent include sulfonate detergents and salicylate detergents. These metallic detergents may be used alone or in combination.

As the sulfonate detergent, the above-described sulfonate detergents may be used. The preferable embodiment of the sulfonate detergent is as described above.

As the salicylate detergent, the above-described salicylate detergent may be used. The preferable embodiment of the salicylate detergent is as described above.

In one preferable embodiment, the component (A2) is a Ca sulfonate detergent and/or a Ca salicylate detergent. The base number of the Ca sulfonate detergent is preferably no less than 10 mgKOH/g, more preferably no less than 150 mgKOH/g, and further preferably no less than 250 mgKOH/g, and preferably no more than 500 mgKOH/g, and more preferably no more than 450mgKOH/g. By having such lower limit values or more of the base number, good acid neutralizing property may be obtained. By having such upper limit values or less of the base number, good detergent property may be obtained. The base number of the Ca salicylate detergent is preferably no less than 60 mgKOH/g, and more preferably no less than 100 mgKOH/g, and preferably no more than 350 mgKOH/g, and more preferably 300 mgKOH/g. By having such lower limit values or more of the base number, good acid neutralizing property may be obtained. By having such upper limit values or less of the base number, good detergent property may be obtained.

### <(B) Demulsifier>

As the (B) demulsifier (hereinafter referred to as "component (B)") in the first embodiment of the lubricating oil composition of the present invention, one or more polyether compound is used. So-called demulsifiers which are commercially available may be used.

As the polyether compound that may be preferably used as the component (B), one or more polyether compound selected from the group consisting of: polyoxypropylene glycol monoalkyl ethers such as polypropylene glycol butyl ether and polypropylene glycol stearyl ether; polyoxyethylene polyoxypropylene alkyl ether (ethylene oxide-propylene oxide copolymer); polyoxyethylene alkyl ether; polyethylene glycol fatty acid ester; polyoxyethylene glycerin fatty acid ester; polyoxyethylene sorbit fatty acid ester; and polyoxyethylene sorbitan fatty acid ester may be given. They may be used alone or in combination.

Among these polyether compounds, polyether compounds including propylene oxide unit are especially preferable, such as: polyoxypropylene glycol monoalkyl ethers such as polypropylene glycol butyl ether and polypropylene glycol stearyl ether; and polyoxyethylene polyoxypropylene alkyl ether (ethylene oxide-propylene oxide copolymer).

The molecular weight of the component (B) is not particularly limited, and preferably no less than 350, more preferably no less than 500, and further preferably no less than 1000, and preferably no more than 30000, more preferably no more than 10000, and further preferably no more than 5000, by number average molecular weight. By having such lower limit values or more of the number average molecular weight of the component (B), good demulsibility may be obtained.

The HLB (hydrophile-lipophile balance) value of the component (B) is not particularly limited as long as it shows demulsification function (emulsion destabilization function), and preferably no less than 13, and more preferably no less than 14.5. The HLB value must be no more than 20 by definition, and preferably no more than 19.5 in view of affinity with the base oil.

The content of the component (B) in the first embodiment of the lubricating oil composition of the present invention is 0.02 to 5 mass% on the basis of the total mass of the composition. The content is preferably no less than 0.03 mass%, more preferably no less than 0.04 mass%, and preferably no more than 4 mass%, and more preferably no more than 3 mass%. By having such lower limit values or more of the content of the component (B), good demulsibility may be obtained.

### <(C) Nitrogen-containing ashless dispersant (1)>

The first embodiment of the lubricating oil composition of the present invention may include (C) a nitrogen-containing ashless dispersant (hereinafter referred to as "component (C)").

As the component (C), for example one or more compound selected from the following (C-1) to (C-3) may be used.
(C-1) a succinimide having at least one alkyl or alkenyl group in a molecule thereof, or a derivative thereof (hereinafter referred to as "component (C-1)");
(C-2) a benzylamine having at least one alkyl or alkenyl group in a molecule thereof, or a derivative thereof (hereinafter referred to as "component (C-2)"); and
(C-3) a polyamine having at least one alkyl or alkenyl group in a molecule thereof, or a derivative thereof (hereinafter referred to as "component (C-3)").

As the component (C), the component (C-1) may be especially preferably used. Examples of the succinimide having at least one alkyl group or alkenyl group in a molecule thereof of the component (C-1) include a compound represented by the following formula (3) or (4).

In the formula (3), R³ is a C₄₀-C₄₀₀ alkyl or alkenyl group, h is an integer of 1 to 5, preferably 2 to 4. The carbon number of R³ is preferably no less than 60 and preferably no more than 350.

In the formula (4), R⁴, independently, same or different, is a C₄₀-C₄₀₀ alkyl or alkenyl group. R⁴ is especially preferably a polybutenyl group. i is an integer of 0 to 4, preferably of 1 to 3. The carbon number of R⁴ is preferably no less than 60 and preferably no more than 350.

By having the above-described lower limit values or more of the carbon numbers of R³ and R⁴ in the formulas (3) and (4), it is possible to obtain good solubility to the lubricating base oil. By having the above-described upper limit values or less of the carbon numbers of R³ and R⁴, it is possible to increase the low-temperature fluidity of the lubricating oil composition.

The alkyl or alkenyl group (R³, R⁴) in the formulas (3) and (4) may be linear or branched. Preferable examples thereof include oligomers of olefins such as propylene, 1-butene and isobutene, and a branched alkyl or alkenyl group derived from a co-oligomer of ethylene and propylene. Among them, a branched alkyl or alkenyl group derived from an oligomer of isobutene idiomatically called as polyisobutylene, and a polybutenyl group are most preferable. A preferable weight-average molecular weight of the alkyl or alkenyl group (R³, R⁴) in the formulas (3) and (4) is 800 to 3500.

The succinimide having at least one alkyl or alkenyl group in a molecule thereof includes a so-called mono-type succinimide represented by the formula (3), in which succinic anhydride is added only to one end of the polyamine chain, and a so-called bis-type succinimide represented by the formula (4), in which succinic anhydride is added to both ends of the polyamine chain. The lubricating oil composition of the present invention may include either one of the mono-type succinimide and the bis-type succinimide, and may include a mixture of the mono-type and bis-type succinimides.

The production method of the succinimide having at least one alkyl or alkenyl group in a molecule thereof is not particularly limited. For example, it may be obtained by reaction of polyamine and an alkyl or alkenyl succinic acid obtained by reaction of a compound having a C₄₀-C₄₀₀ alkyl or alkenyl group and maleic anhydride at 100 to 200°C. Here, examples of the polyamine include diethylenetriamine, triethylenetetramine, tetraethylenepentamine and pentaethylenehexamine.

Examples of the benzylamine having at least one alkyl or alkenyl group in a molecule thereof of the component (C-2) include a compound represented by the following formula (5).

In the formula (5), R⁵ is a C₄₀ to C₄₀₀ alkyl or alkenyl group, j is an integer of 1 to 5, preferably 2 to 4. The carbon number of R⁵ is preferably no less than 60 and preferably no more than 350.

The production method of the component (C-2) is not particularly limited. For example, the method of reacting a propylene oligomer, polybutene or polyolefin such as ethylene-α-olefin copolymer with phenol to make an alkylphenol, thereafter reacting the alkylphenol with formaldehyde and a polyamine such as diethylenetriamine, triethylenetetramine, tetraethylenepentamine, and pentaethylenehexamine by Mannich reaction may be given.

Examples of the polyamine having at least one alkyl or alkenyl group in a molecule thereof of the component (C-3) include a compound represented by the following formula (6).

R⁶-NH-(CH₂CH₂NH)ₖ-H (6)

In the formula (6), R⁶ is a C₄₀ to C₄₀₀ alkyl or alkenyl group, and k is an integer of 1 to 5, preferably 2 to 4. The carbon number of R⁶ is preferably no less than 60 and preferably no more than 350.

The production method of the component (C-3) is not particularly limited. For example, a method of: chlorinating a propylene oligomer, polybutene or polyolefin such as ethylene-α-olefin copolymer; thereafter reacting the chlorinated product with a polyamine such as ammonia, ethylenediamine, diethylenetriamine, triethylenetetramine, tetraethylenepentamine, and pentaethylenehexamine may be given.

As the derivative in the components (C-1) to (C-3), for example, (i) a modified compound by an oxygen-containing organic compound, in which some or all of the remaining amino group and/or imino group is neutralized or amidated by a function of C₁-C₃₀ monocarboxylic acid such as fatty acid, C₂-C₃₀ polycarboxylic acid (e.g. oxalic acid, phthalic acid, trimellitic acid, and pyromellitic acid), anhydrides or ester compounds thereof, C₂-C₆ polyalkylene oxide, or hydroxyl(poly)oxyalkylenecarbonate to the above-described succinimide having at least one alkyl or alkenyl group in a molecule thereof (hereinafter referred to as "above-described nitrogen-containing compound"); (ii) a boron modified compound in which some or all of the remaining amino group and/or imino group is neutralized or amidated by a function of boric acid to the above-described nitrogen-containing compound; (iii) a phosphoric-acid modified compound in which some or all of the remaining amino group and/or imino group is neutralized or amidated by a function of phosphoric acid to the above-described nitrogen-containing compound; (iv) a sulfur modified compound obtained by a function of a sulfur compound to the above-described nitrogen-containing compound; and (v) a modified compound obtained by carrying out two or more modifications in combination selected from a modification by an oxygen-containing organic compound, boron modification, phosphoric acid modification, and sulfur modification, to the above-described nitrogen-containing compound may be given. Among the derivatives of (i) to (v), by using a boron modified compound of alkenyl succinimide, especially a boron modified compound of a bis-type alkenyl succinimide, it is possible to further improve the heat resistance of the lubricating oil composition.

The molecular weight of the component (C) is not particularly limited, and a preferable weight-average molecular weight the component (C) is from 1000 to 8000. In the first embodiment of the lubricating oil composition of the present invention, the content of the component (C) when contained is no more than 0.2 mass%, preferably no less than 0.02 mass%, more preferably no less than 0.04 mass%, and further preferably no less than 0.07 mass%, and preferably no more than 0.12 mass%, in terms of nitrogen on the basis of the total mass of the lubricating oil composition. By having the above-described lower limit values or more of the content of the component (C), it is possible to sufficiently improve the coking resistance (heat resistance) of the lubricating oil composition. By having the above-described upper limit values or less of the content of the component (C), it is possible to obtain good separation property of impurities in a centrifugal cleaner and to improve water separation property to inhibit the scum generation in the scrubber.

### <(C) Nitrogen-containing ashless dispersant (2)>

The second embodiment of the lubricating oil composition of the present invention optionally includes (C-1') a succinimide having at least one alkyl or alkenyl group in a molecule thereof, or a borated derivative thereof (hereinafter may be referred to as "component (C-1')"). However, when the second embodiment of the lubricating oil composition of the present invention includes the component (C-1'), the content of the component (C-1') has to be no more than 0.015 mass% in terms of nitrogen on the basis of the total mass of the composition. By having the content of the component (C-1') of no more than 0.015 mass% in terms of nitrogen, good demulsibility may be obtained and the generation of scum in the scrubber may be inhibited.

Examples of the succinimide having at least one alkyl or alkenyl group in a molecule thereof include the compounds represented by the above formulas (3) or (4) described above regarding the component (C-1) in the first embodiment. The preferable embodiments of these compounds are as described above.

Examples of the borated derivative of the succinimide having at least one alkyl or alkenyl group in a molecule thereof include a so-called boron modified compound in which some or all of the remaining amino group and/or imino group is neutralized or amidated by reaction of boric acid with the above-described succinimide having at least one alkyl or alkenyl group in a molecule thereof.

The molecular weight of the component (C-1') is not particularly limited, and a preferable weight-average molecular weight thereof is from 1000 to 8000.

### <Other additive>

The lubricating oil composition of the present invention may further contain any additives generally used in lubricating oils, depending on the intended use. Examples of such additives include zinc dithiophosphates, antioxidants, defoaming agents, pour point depressants, metal inactivators, and extreme pressure agents.

As the zinc dithiophosphate (ZnDTP), a compound represented by the following formula (7) may be preferably used.

In the formula (7), R⁷ independently, the same or different, is a C₁-C₂₄ hydrocarbon group. Preferable examples of the C₁-C₂₄ hydrocarbon group include a linear or branched C₁-C₂₄ alkyl group. The carbon number of R⁷ is preferably no less than 3, and preferably no more than 12, and more preferably no more than 8. The alkyl group as R⁷ may be any one of a primary alkyl group, a secondary alkyl group, and a tertiary alkyl group. The alkyl group as R⁷ is preferably a primary alkyl group or a secondary alkyl group or a mixture thereof, and most preferably a primary alkyl group.

Examples of the above zinc dithiophosphate include: zinc dialkyldithiophosphates having a linear or branched C₃-C₁₈, preferably C₃-C₁₀ alkyl group (primary, secondary or tertiary, preferably primary or secondary), such as zinc dipropyl dithiophosphate, zinc dibutyl dithiophosphate, zinc dipentyl dithiophosphate, zinc dihexyl dithiophosphate, zinc diheptyl dithiophosphate, and zinc dioctyl dithiophosphate; zinc di((alkyl)aryl)dithiophosphates having a C₆-C₁₈, preferably C₆-C₁₀ aryl or alkyaryl group, such as zinc diphenyl dithiophosphate and zinc ditolyl dithiophosphate; and a mixture of two or more thereof.

The production method of the above zinc dithiophosphate is not particularly limited. For example, it may be synthesized by making a reaction of an alcohol having an alkyl group corresponding to R⁷ with phosphorus pentasulfide to synthesize a dithiophosphoric acid, and neutralizing the dithiophosphoric acid by zinc oxide.

In the lubricating oil composition of the present invention, the content of the zinc dithiophosphate is preferably 0.03 to 1.0 mass%, more preferably 0.05 to 0.5 mass%, and especially preferably 0.01 to 0.3 mass% on the basis of the total mass of the composition. The zinc dithiophosphate is desirably contained in such a manner that the phosphorus component in the lubricating oil composition is preferably 25 to 700 mass ppm, more preferably no less than 40 mass ppm, further preferably no less than 50 mass ppm, and especially preferably no less than 80 mass ppm, and more preferably no more than 500 mass ppm, further preferably no more than 300 mass ppm, and especially preferably no more than 250 mass ppm. If the phosphorus component derived from the zinc dithiophosphate in the lubricating oil composition is no less than 25 mass ppm, it is possible to secure necessary oxidation stability, and if it is no more than 700 mass ppm, it is possible to prevent the base number from lowering due to hydrolysis of the zinc dithiophosphate.

Examples of the antioxidant include ashless antioxidants such as phenol-based antioxidants, amine-based antioxidants, and metallic antioxidants. Among them, phenol-based antioxidants and/or amine-based antioxidants are preferably used, in view of maintaining high temperature detergent performance. When an antioxidant is contained in the lubricating oil composition of the present invention, the content thereof is preferably no less than 0.05 mass%, and more preferably no less than 0.1 mass%, on the basis of the total mass of the composition, and when the antioxidant is an amine-based antioxidant, the content is especially preferably no less than 0.3 mass%, and when the antioxidant is a phenol-based antioxidant, the content is especially preferably no less than 0.15 mass%, on the basis of the total mass of the composition. The upper limit of the content of the antioxidant is not particularly limited, and preferably no more than 5 mass% and more preferably no more than 2 mass% on the basis of the total mass of the composition.

Examples of the defoaming agent include silicone oils, derivatives of alkenyl succinic acid, esters of aliphatic polyhydroxy alcohol and a long-chain fatty acid, methyl salicylate and o-hydroxybenzyl alcohol, aluminum stearate, potassium oleate, N-dialkyl-allylaminenitroaminoalkanol, aromatic amine salts of isoamyl octyl phosphate, alkylalkylenediphosphate, metal derivatives of thioethers, metal derivatives of disulfides, fluorine compounds of aliphatic hydrocarbons, triethylsilane, dichlorosilane, alkylphenyl polyethylene glycol ethersulfide, and fluoroalkylether. When a defoaming agent is contained in the lubricating oil composition of the present invention, the content thereof is normally 0.0005 to 1 mass% on the basis of the total mass of the composition. When the defoaming agent includes silicon, the defoaming agent is preferably included in such a manner that the Si component in the lubricating oil composition is 5 to 50 mass ppm.

Examples of the pour point depressant include polymethacrylate-based polymers that conform to the lubricating base oil to be used. When a pour point depressant is contained in the lubricating oil composition of the present invention, the content thereof may be normally 0.005 to 5 mass% on the basis of the total mass of the composition.

Examples of the metal deactivator include imidazoline, pyrimidine derivatives, alkylthiadiazole, mercaptobenzothiazole, benzotriazole or derivatives thereof, 1,3,4-thiadiazolepolysulfide, 1,3,4-thiadiazolyl-2,5-bisdialkyldithiocarbamate, 2-(alkyldithio)benzoimidazole, and β-(o-carboxybenzylthio)propionitrile. When a metal deactivator is contained in the lubricating oil composition of the present invention, the content thereof is normally 0.005 to 1 mass% on the basis of the total mass of the composition.

Examples of the extreme-pressure agent include sulfur-based, phosphorus-based, and sulfur-phosphorus-based extreme-pressure agents. Specific examples thereof include phosphorous esters, thiophosphorous esters, dithiophosphorous esters, trithiophosphorous esters, phosphate esters, thiophosphate esters, dithiophosphate esters, trithiophosphate esters, amine salts thereof, metallic salts thereof, derivatives thereof, dithiocarbamate, zinc dithiocarbamate, molybdenum dithiocarbamate, disulfides, polysulfides, olefin sulfides, and sulfurized oils and fats. When an extreme-pressure agent is contained in the lubricating oil composition of the present invention, the content thereof is not particularly limited, and normally 0.01 to 5 mass% on the basis of the total mass of the composition.

### <Lubricating oil composition>

The base number of the lubricating oil composition of the present invention is 15 to 125 mgKOH/g, preferably no less than 20 mgKOH/g, more preferably no less than 30 mgKOH/g, and further preferably no less than 40 mgKOH/g, and preferably no more than 120 mgKOH/g, more preferably no more than 105 mgKOH/g, and further preferably no more than 100 mgKOH/g. If the base number of the lubricating oil composition is less than 15 mgKOH/g, the detergency might be insufficient. If the base number of the lubricating oil composition is more than 125 mgKOH/g, excessive base components accumulate on the piston to obstruct formation of oil film, which results in a potential bore polish and scuffing. Therefore it is not preferable that the base number of the lubricating oil composition is less than 15 mgKOH/g or more than 125 mgKOH/g.

The kinematic viscosity at 100°C of the lubricating oil composition of the present invention is 10 to 30 mm²/s, preferably no less than 12 mm²/s, more preferably no less than 12.5 mm²/s, further preferably no less than 16.3 mm²/s, and especially preferably no less than 18.0 mm²/s, and preferably no more than 27 mm²/s, more preferably no more than 26.1 mm²/s, further preferably no more than 21.9 mm²/s, and especially preferably no more than 21.0 mm²/s. If the kinematic viscosity at 100°C of the lubricating oil composition is less than 10 mm²/s, the performance of oil formation is insufficient, which might results in searing of ring and liner. Therefore, it is not preferable that the kinematic viscosity at 100°C of the lubricating oil composition of the present invention is less than 10 mm²/s. If the kinematic viscosity at 100°C of the lubricating oil composition is more than 30 mm²/s, which is a high viscosity, the starting performance might degrade. Therefore it is not preferable that the kinematic viscosity at 100°C of the lubricating oil composition of the present invention is more than 30 mm²/s.

In the second embodiment of the lubricating oil composition of the present invention, the Ph value represented by the following formula (1) is no more than 20 × 10⁻³, preferably no more than 19 × 10⁻³, and more preferably no more than 18 × 10⁻³. By having such an upper limit value or less of the Ph value, the demulsibility improves, and it is possible to inhibit generation of scum in the scrubber. $Ph value = {C}_{Ca} \times 2 / \left({r}_{M}\times 40.08\right)$ (in the formula (1), C_{Ca} represents calcium content (mass%) derived from the component (A1), and r_{M} represents a metal ratio of the component (A1).)

The calcium content (mass%) derived from the component (A1) mentioned here means a value of the content of calcium derived from the Ca phenate detergent of the component (A1) in the lubricating oil composition of the present invention, show by mass% on the basis of the total mass of the lubricating oil composition. The metal ratio of the component (A1) mentioned here is a value calculated according to the following formula, regarding the Ca phenate detergent which is the component (A1). $\begin{matrix}Metal ratio of component \left(A1\right) = calcium content \left(mass%\right) in Ca phenate detergent \\ which is component \left(A1\right) / calcium content \left(mass %\right) derived from soap base in Ca phenate \\ detergent which is component \left(A1\right)\end{matrix}$

### <Method of lubricating cylinder>

The method of lubricating a cylinder of a crosshead diesel engine equipped with a scrubber according to the second aspect of the present invention includes: (i) operating the crosshead diesel engine while supplying the lubricating oil composition according to the first aspect of the present invention to the cylinder of the crosshead diesel engine equipped with a scrubber; and (ii) purifying at least a part of gas exhausted from the cylinder in the scrubber.

As the crosshead diesel engine equipped with a scrubber, known crosshead diesel engines equipped with scrubbers may be used without particular limitations (for example, see Patent Literatures 1 to 5). The method of supplying the lubricating oil composition according to the first aspect of the present invention to the crosshead diesel engine is not particularly limited, and known methods for supplying lubricating oils to crosshead diesel engines may be used. The scrubber may be an EGR scrubber, may be a scrubber that does not send back the gases that passed through the scrubber to the inlet side but releases them to the environment, and may be a combination thereof. However, considering that the demulsibility improved in the lubricating oil composition according to the first aspect of the present invention advantageously functions, a scrubber that purifies gasses guided in the scrubber by making the gasses into contact with water and/or a basic aqueous solution is preferable. As the basic aqueous solution, an aqueous solution in which salts such as alkali metal hydroxides and alkali metal carbonates are dissolved may be used for example, and seawater may be preferably used.

### Examples

Hereinafter, the present invention will be explained further in detail based on Examples and Comparative Examples. However, the present invention is not limited to these Examples.

### <Examples 1 to 11, Comparative Examples 1 to 7>

Regarding the first embodiment of the lubricating oil composition, lubricating oil compositions of compounding formulations shown in Tables 1 and 2 were prepared and a high-speed emulsification test was carried out thereon. The results are shown in Tables 1 and 2. In Tables 1 and 2, the amounts of the base oils are the contents on the basis of the total amount of the base oils, and the amounts of additives are the contents on the basis of the total amount of the composition.

### (Commercially available cylinder oil)

A commercially available cylinder oil containing: mineral base oil in an amount of 81 mass%; a Ca phenate detergent of the above formula (1) wherein R¹ is a C₁₂ alkyl or alkenyl group; a carbonic Ca sulfonate detergent (C₂₀, C₂₂ and C₂₄ hydrocarbon groups are bonded to an aromatic six-membered ring); a polybutenyl succinimide of the above formula (4) wherein R⁴ is a polybutenyl group; alkyldiphenylamine (carbon numbers of the alkyl groups are 4 and 8); alkylphenol; and a Si compound. The calcium content of the commercially available cylinder oil was 2.60 mass% in terms of calcium on the basis of the total mass of the commercially available cylinder oil. The nitrogen content of the commercially available cylinder oil was 0.03 mass% in terms of nitrogen on the basis of the total mass of the commercially available cylinder oil.

### (Base oil)

Base oil 1: solvent refining oil, 500 N, kinematic viscosity at 100°C 10.8 mm²/s, content of saturated component 62 mass%
Base oil 2; solvent refining oil, Bright Stock, kinematic viscosity at 100°C 31.8 mm²/s, content of saturated component 46 mass%

### (Metallic detergent)

Ca phenate: a Ca phenate of the above formula (1) wherein A is a sulfide group, x = 1 to 2, m = 1 to 2, base number 250 mgKOH/g, Ca content 8.9 mass%, metal ratio 4.5, sulfur component 3.5 mass%
Ca sulfonate: base number 400 mgKOH/g, Ca content 15.5 mass%, metal ratio 20

### (Nitorogen-containing ashless dispersant)

Nitrogen-containing ashless dispersant: a polyisobutenyl succinimide of the above formula (4) wherein R⁴ is a polybutenyl group, n = 5, N content 1.1 mass%, Mw = 2490, weight average molecular weight of the part of the polybutenyl group Mw = 1000

### (Demulsifier)

B-1: polypropylene glycol stearyl ether, Mw = 1600
B-2: polypropylene glycol butyl ether ("NEWPOL LB-285" manufactured by Sanyo Chemical Industries, Ltd.), Mn = 1170
B-3: polypropylene glycol butyl ether ("NEWPOL LB-1715" manufactured by Sanyo Chemical Industries, Ltd.), Mn = 2390
B-4: ethylene oxide-propylene oxide copolymer, Mw = 4840

### Solbitan monooleate: HLB4.3

### <Evaluation method>

### (High-speed emulsification test)

This test was a model examination simulating a process of oil-water separation after stirring in a scrubber. In a 100 ml measuring cylinder, 40 g of a sodium hydroxide aqueous solution (pH = 12) and 10 g of the sample oil were collected. The measuring cylinder was set on a homogenizer (POLYTRON PT10-35, generator shaft PT36/4K manufactured by KINEMATICA), and stirred for 5 minutes at 15,000 rpm. After that, the homogenizer was pulled upward from the measuring cylinder and allowed to stand for 5 minutes, to collect the wet, oil and emulsion attached to the homogenizer to the measuring cylinder. The measuring cylinder after the test was allowed to stand for 1 week at a room temperature. From the separated oil amount, the separation performance was judged as follows.
Separated oil amount of 10 ml: mark 3,
Separated oil amount of no less than 7.5 ml and less than 10 ml: mark 2.5,
Separated oil amount of no less than 5 ml and less than 7.5 ml: mark 2,
Separated oil amount of no less than 1 ml and less than 5 ml: mark 1, and
Separated oil amount of less than 1 ml: mark 0
Oils of mark no less than 2 were acceptable and no more than 1 were rejected.

### <Evaluation result>

The lubricating oil compositions of Examples 1 to 11 showed good separation performances on the high-speed emulsification test (Table 1). The compositions of Comparative Examples 1 and 5 to 7 that did not include the component (B), the composition of Comparative Example 2 including the component (B) by less than 0.02 mass%, and the compositions of Comparative Examples 3 and 4 including surfactants that did not have demulsification function instead of the component (B) each got mark 0 (rejected) in the high-speed emulsification test, which meant they were inferior in separation performance (Table 2). It is noted, when the composition of Comparative Example 1 (that is, the commercially available cylinder oil itself), which marked 0 on the high-speed emulsification test, was used as a cylinder lubricating oil to operate a crosshead diesel engine, and when the exhaust gas was cleaned by a scrubber, scums were generated in the scrubber.

**[Table 1]**

| | | Example 1 | Example 2 | Example 3 | Example 4 | Example 5 | Example 6 | Example 7 | Example 8 | Example 9 | Example 10 | Example 11 |
|---|---|---|---|---|---|---|---|---|---|---|---|---|
| Commercially available cylinder oil | mass% | 99.95 | 99.9 | 99.5 | 99 | 98 | 99.5 | 99.5 | 99.5 | - | - | - |
| Base oil 1 | mass% | | | | | | | | | 41.2 | 39.3 | 43.2 |
| Base oil 2 | mass% | | | | | | | | | 40.5 | 34.9 | 21.3 |
| Ca phenate mass% | | | | | | | | | | 14 | 14 | 20 |
| Ca sulfonate | mass% | | | | | | | | | 1.3 | 8.8 | 12.5 |
| Nitrogen-containing ashless dispersant | mass% | | | | | | | | | 2.7 | 2.7 | 2.7 |
| B-1 -B-1 mas% | mass% | 0.05 | 0.1 | 0.5 | 1 | 2 | | | | | | 0.3 |
| B-2 | mass% | | | | | | 0.5 | | | 0.3 | | |
| B-3 | mass% | | | | | | | 0.5 | | | 0.3 | |
| B-4 | mass% | | | | | | | | 0.5 | | | |
| Solbitan monooleate | mass% | | | | | | | | | | | |
| Methyl oleate | mass% | | | | | | | | | | | |
| Kinematic viscosity of composition (100°C) | mm²/s | 20.7 | 20.7 | 20.7 | 20.7 | 20.7 | 20.7 | 20.7 | 20.7 | 20.5 | 20.5 | 20.5 |
| Base number of composition | mgKOH/g | 70 | 70 | 70 | 70 | 70 | 70 | 70 | 70 | 40 | 70 | 100 |
| Ca content in composition | mass% | 2.6 | 2.6 | 2.6 | 2.6 | 2.6 | 2.6 | 2.6 | 2.6 | 1.4 | 2.6 | 3.7 |
| Nitrogen content in composition | mass% | 0.03 | 0.03 | 0.03 | 0.03 | 0.03 | 0.03 | 0.03 | 0.03 | 0.03 | 0.03 | 0.03 |
| High-speed emulsification test | Mark | 3 | 3 | 3 | 3 | 3 | 2.5 | 3 | 3 | 3 | 3 | 3 |

**[Table 2]**

| | | Comparative Example 1 | Comparative Example 2 | Comparative Example 3 | Comparative Example 4 | Comparative Example 5 | Comparative Example 6 | Comparative Example 7 |
|---|---|---|---|---|---|---|---|---|
| Commercially available cylinder oil | mass% | 100 | 99.99 | 99.5 | 99.5 | - | - | - |
| Base oil 1 | mass% | | | | | 41 | 39.5 | 43.4 |
| Base oil 2 | mass% | | | | | 41 | 35 | 21.4 |
| Ca phenate | mass% | | | | | 14 | 14 | 20 |
| Ca sulfonate | mass% | | | | | 1.3 | 8.8 | 12.5 |
| Nitrogen-containing ashless dispersant | mass% | | | | | 2.7 | 2.7 | 2.7 |
| B-1 | mass% | | 0.01 | | | | | |
| B-2 | mass% | | | | | | | |
| B-3 | mass% | | | | | | | |
| B-4 | mass% | | | | | | | |
| Solbitan monooleate | mass% | | | 0.5 | | | | |
| Methvl oleate | mass% | | | | 0.5 | | | |
| Kinematic viscosity of composition (100°C) | mm²/s | 20.7 | 20.7 | 20.7 | 20.7 | 20.5 | 20.5 | 20.5 |
| Base number of composition | mgKOH/g | 70 | 70 | 70 | 70 | 40 | 70 | 100 |
| Ca content in composition | mass% | 2.60 | 2.60 | 2.60 | 2.60 | 1.4 | 2.6 | 3.7 |
| Nitrogen content in composition | mass% | 0.03 | 0.03 | 0.03 | 0.03 | 0.03 | 0.03 | 0.03 |
| High-speed emulsification test | Mark | 0 | 0 | 0 | 0 | 0 | 0 | 0 |

### <Examples 12 to 26, Comparative Examples 8 to 13>

Regarding the second embodiment of the lubricating oil composition of the present invention, lubricating oil compositions of the compounding formulations shown in Tables 3 to 5 were prepared, and a high-speed emulsification test was carried out in the same way as above. The results ar shown in Tables 3 to 5. In Tables 3 to 5, the amounts of the base oils are the contents on the basis of the total amount of the base oils, and the amounts of additives are the contents on the basis of the total amount of the composition.

### (Base oil)

Base oil 1: solvent refining base oil, 500 N, kinematic viscosity at 100°C 10.8 mm²/s, content of saturated component 62 mass%
Base oil 2: solvent refining base oil, Bright Stock, kinematic viscosity at 100°C 31.8 mm²/s, content of saturated component 46 mass%

### (Component (A1))

(A1)-1: a Ca phenate of the above formula (1) wherein A is a sulfide group, x = 1 to 2, and m = 1 to 2, base number 250 mgKOH/g, Ca content 8.9 mass%, metal ratio 4.5, sulfur content 3.5 mass%
(A1)-2: a Ca phenate of the above formula (1) wherein A is a sulfide group, x = 1 to 3, and m = 1 to 4, base number 150 mgKOH/g, Ca content 5.4 mass%, metal ratio 2.7, sulfur content 4.1 mass%
(A1)-3: a Ca phenate of the above formula (1) wherein A is a methylene group, x = 1 to 3, and m = 1 to 4, base number 70 mgKOH/g, Ca content 2.5 mass%, metal ratio 1.3

### (Component (A2))

(A2)-1: a Ca sulfonate, base number 400 mgKOH/g, Ca content 15.5 mass%, metal ratio 20
(A2)-2: a Ca salicylate of the above formula (2) wherein M is calcium, R² is a C₁₄-C₁₈ alkyl group derived from α olefin, and n = 1 to 2, base number 225 mgKOH/g, Ca content 8.2 mass%, metal ratio 3.1

### (Component (C-1'))

(C-1')-1: a polyisobutenyl succinimide of the above formula (4) wherein R⁴ is a polybutenyl group and n = 5, bis-type, N content 1.1 mass%, Mw = 2490, weight average molecular weight of the part of the polybutenyl group Mw = 1000
(C-1')-2: a polyisobutenyl succinimide of the above formula (3) wherein R³ is a polybutenyl group, and n = 4, mono-type, N content 2.0 mass%, Mw = 1000

### <Evaluation result>

The lubricating oil compositions of Examples 12 to 26 showed good separation property at the high-speed emulsification test (Tables 1 and 2). The lubricating oil compositions of Examples 24 to 26 showed sufficient demulsification property even though each composition contained the component (C), which functioned as a dispersant, in an amount of no more than 0.015 mass% in terms of nitrogen on the basis of the total mass of the composition. The compositions of Comparative Examples 8 to 10, whose Ph value was over 20 × 10⁻³, each marked 0 (rejected) at the high-speed emulsification test, which meant they were inferior in separation property. The compositions of Comparative Examples 11 to 13, whose content of the component (C) was over 0.015 mass% in terms of nitrogen on the basis of the total mass of the composition, each marked 0 (rejected) at the high-speed emulsification test even though the Ph value was no more than 20 × 10⁻³, which meant they were inferior in separation property.

**[Table 3]**

| | | | Example 12 | Example 13 | Example 14 | Example 15 | Example 16 | Example 17 | Example 18 |
|---|---|---|---|---|---|---|---|---|---|
| Base oil 1 | | mass% | 46.6 | 48.2 | 49.8 | 51.4 | 53.0 | 46.5 | 49.4 |
| Base oil 2 | | mass% | 53.4 | 51.8 | 50.2 | 48.6 | 47.0 | 53.5 | 50.6 |
| (A1)-1 | | mass% | 2.8 | 5.6 | 8.4 | 11.2 | 14.0 | | |
| mass% | | | | | | | | 3.5 | 10.3 |
| (A1)-3 | | mass% | | | | | | | |
| (A2)-1 | | mass% | 15.8 | 14.0 | 12.3 | 10.5 | 8.8 | 16.2 | 13.7 |
| (A2)-2 | | mass% | | | | | | | |
| (C1')-1 | | mass% | | | | | | | |
| (C-1')-2 | | mass% | | | | | | | |
| Lubricating oil composition | | | | | | | | | |
| | Base number | mgKOH/g | 70 | 70 | 70 | 70 | 70 | 70 | 70 |
| | Kinematic viscosity (100°C) | mm²/s | 20.5 | 20.5 | 20.5 | 20.5 | 20.5 | 20.5 | 20.5 |
| | Ca component | mass% | 2.70 | 2.67 | 2.65 | 2.62 | 2.61 | 2.70 | 2.68 |
| | Ca component derived from Ca phenate | mass% | 0.250 | 0.500 | 0.750 | 1.000 | 1.250 | 0.189 | 0.556 |
| | Nitrogen component derived from component (C-1') | mass% | 0 | 0 | 0 | 0 | 0 | 0 | 0 |
| Ph value×10³ | | | 2.763 | 5.527 | 8.290 | 11.053 | 13.817 | 3.493 | 10.279 |
| High-speed emulsification test | | Mark | 2 | 3 | 3 | 3 | 3 | 2 | 3 |

**[Table 4]**

| | | | Example 19 | Example 20 | Example 21 | Example 22 | Example 23 | Example 24 | Example 25 | Example 26 |
|---|---|---|---|---|---|---|---|---|---|---|
| Base oil 1 | | mass% | 52.2 | 51.6 | 56.0 | 53.0 | 49.4 | 49.8 | 49.8 | 49.8 |
| Base oil 2 | | mass% | 47.8 | 48.4 | 44.0 | 47.0 | 50.6 | 50.2 | 50.2 | 50.2 |
| (A1)-1 | | mass% | | | | 14.0 | | 8.4 | 8.4 | 8.4 |
| (A1)-2 | | mass% | 16.9 | | | | 10.3 | | | |
| (A1)-3 | | mass% | | 9.0 | 15.0 | | | | | |
| | | mass% | 11.2 | 16.0 | 15.0 | | 7.5 | 12.3 | 12.3 | 12.3 |
| (A2)-2 | | mass% | | | | 15.6 | 11.0 | | | |
| (C-1')-1 | | mass% | | | | | | 0.5 | 1.0 | |
| (C-1')-2 | | mass% | | | | | | | | 0.5 |
| | Lubricating oil composition | | | | | | | | | |
| | Base number | mgKOH/g | 70 | 70 | 70 | 70 | 70 | 70 | 70 | 70 |
| | Kinematic viscosity (100°C) | mm²/s | 20.5 | 20.5 | 20.5 | 20.5 | 20.5 | 20.5 | 20.5 | 20.5 |
| | Ca component | mass% | 2.65 | 2.71 | 2.70 | 2.53 | 2.62 | 2.65 | 2.65 | 2.65 |
| | Ca component derived from Ca phenate | mass% | 0.913 | 0.230 | 0.380 | 1.250 | 0.556 | 0.750 | 0.750 | 0.750 |
| | Nitrogen component derived from component (C-1') | mass% | 0.000 | 0.000 | 0.000 | 0.000 | 0.000 | 0.005 | 0.011 | 0.010 |
| Ph value×10³ | | | 16.866 | 8.637 | 14.394 | 13.817 | 10.279 | 8.290 | 8.290 | 8.290 |
| High-speed emulsification test | | Mark | 3 | 3 | 3 | 3 | 3 | 3 | 2 | 2 |

**[Table 5]**

| | | | Comparative Example 8 | Comparative Example 9 | Comparative Example 10 | Comparative Example 11 | Comparative Example 12 | Comparative Example 13 |
|---|---|---|---|---|---|---|---|---|
| Base oil 1 | | mass% | 57.0 | 56.9 | 61.5 | 49.8 | 49.8 | 49.8 |
| Base oil 2 | | mass% | 43.0 | 43.1 | 38.5 | 50.2 | 50.2 | 50.2 |
| (A1)-1 | | mass% | 21.0 | | | 8.4 | 8.4 | 8.4 |
| (A1)-2 | | mass% | | 28.0 | | | | |
| (A1)-3 | | mass% | | | 22.5 | | | |
| (A2)-1 | | mass% | 4.4 | 7.0 | 13.8 | 12.3 | 12.3 | 12.3 |
| (A2)-2 | | mass% | | | | | | |
| (C-1') | | mass% | | | | 1.5 | | |
| (C-1')-2 | | mass% | | | | | 1.0 | 1.5 |
| Lubricating oil composition | | | | | | | | |
| | Base number | mgKOH/g | 70 | 70 | 70 | 70 | 70 | 70 |
| | Kinematic viscosity (100°C) | mm²/s | 20.5 | 20.5 | 20.5 | 20.5 | 20.5 | 20.5 |
| | Ca component | mass% | 2.55 | 2.60 | 2.70 | 2.65 | 2.65 | 2.65 |
| | Ca component derived from Ca phenate | mass% | 1.87 | 1.51 | 0.563 | 0.750 | 0.750 | 0.750 |
| | Nitrogen component derived from component (C-1') | mass% | 0.000 | 0.000 | 0.000 | 0.016 | 0.020 | 0.030 |
| Ph value×10³ | | | 20.725 | 27.944 | 21.591 | 8.290 | 8.290 | 8.290 |
| High-speed emulsification test | | Mark | 0 | 0 | 0 | 0 | 0 | 0 |

## Claims

1. A cylinder lubricating oil composition for a crosshead diesel engine equipped with a scrubber, comprising:
a base oil; and
(A) a metallic detergent,
wherein the lubricating oil composition has a base number measured by the perchloric acid method of 15 to 125 mgKOH/g, and a kinematic viscosity at 100°C of 10 to 30 mm²/s; and
wherein the lubricating oil composition comprises, as the component (A),
(A1) a Ca phenate detergent; and
(A2) a metallic detergent other than any Ca phenate detergent;
the lubricating oil composition optionally comprises:
(C-1') a succinimide having at least one alkyl or alkenyl group in a molecule thereof, or a borated derivative thereof, in an amount of no more than 0.015 mass% in terms of nitrogen on the basis of the total mass of the composition; and
wherein a Ph value represented by the following formula (1) is no more than 20 × 10⁻³: $Ph value = {C}_{Ca} \times 2 / \left({r}_{M}\times 40.08\right)$ wherein in the formula (1), C_{Ca} represents calcium content in mass% derived from the component (A1), and r_{M} represents a metal ratio of the component (A1); and
wherein the metal ratio of component (A1) is calculated by the following formula (2): $\begin{matrix}metal ratio of component \left(A1\right) = calcium content in mass % in Ca phenate detergent \\ which is component \left(A1\right) / calcium content in mass % derived from soap base in Ca phenate \\ detergent which is component \left(A1\right)\end{matrix}$

2. The cylinder lubricating oil composition for the crosshead diesel engine equipped with the scrubber according to claim 1,
wherein the lubricating oil composition comprises the component (C-1') in an amount of greater than 0 mass% and no more than 0.015 mass% in terms of nitrogen on the basis of the total mass of the composition.

3. The cylinder lubricating oil composition for the crosshead diesel engine equipped with the scrubber according to claim 1 or 2,
wherein the component (A2) is a Ca sulfonate and/or a Ca salicylate.

4. A method of lubricating a cylinder of a crosshead diesel engine equipped with a scrubber, comprising:
operating the crosshead diesel engine while supplying the lubricating oil composition as in any one of claims 1 to 3 to the cylinder of the crosshead diesel engine equipped with the scrubber; and
purifying at least a part of gas exhausted from the cylinder in the scrubber.

5. The method of lubricating the cylinder of the crosshead diesel engine equipped with the scrubber according to claim 4,
wherein the purifying in the scrubber comprises contacting the gas introduced into the scrubber with water and/or a basic aqueous solution.

6. A cylinder lubricating oil composition for a crosshead diesel engine equipped with a scrubber, comprising:
a base oil;
(A) a metallic detergent, and
(B) a demulsifier in an amount of 0.02 to 5.0 mass% on the basis of the total mass of the composition, wherein the component (B) is one or more polyether compound.
wherein the lubricating oil composition optionally comprises:
(C) a nitrogen-containing ashless dispersant in an amount of no more than 0.2 mass% in terms of nitrogen on the basis of the total mass of the composition,
wherein the lubricating oil composition has a base number measured by the perchloric acid method of 15 to 125 mgKOH/g, and a kinematic viscosity at 100°C of 10 to 30 mm²/s.

7. The cylinder lubricating oil composition for the crosshead diesel engine equipped with the scrubber according to claim 6,
wherein the lubricating oil composition optionally comprises:
(C) the nitrogen-containing ashless dispersant in an amount of no more than 0.12 mass% in terms of nitrogen on the basis of the total mass of the composition,

8. The cylinder lubricating oil composition for the crosshead diesel engine equipped with the scrubber according to claim 6 or 7,
wherein the lubricating oil composition comprises:
(C) the nitrogen-containing ashless dispersant.

9. The cylinder lubricating oil composition for the crosshead diesel engine equipped with the scrubber according to any one of claims 6 to 8,
wherein a number average molecular weight of the component (B) is no less than 500.

10. The cylinder lubricating oil composition for the crosshead diesel engine equipped with the scrubber according to any one of claims 6 to 9,
wherein the component (A) is a Ca phenate.

11. A method of lubricating a cylinder of a crosshead diesel engine equipped with a scrubber, comprising:
operating the crosshead diesel engine while supplying the lubricating oil composition as in any one of claims 6 to 10 to the cylinder of the crosshead diesel engine equipped with the scrubber; and
purifying at least a part of gas exhausted from the cylinder in the scrubber.

12. The method of lubricating the cylinder of the crosshead diesel engine equipped with the scrubber according to claim 11,
wherein the purifying in the scrubber comprises contacting the gas introduced into the scrubber with water and/or a basic aqueous solution.

## Patentansprüche

1. Zylinder-Schmiermittelölzusammensetzung für einen Kreuzkopfdieselmotor, ausgerüstet mit einem Gaswäscher, enthaltend:
ein Grundöl und
(A) ein metallisches Reinigungsmittel,
worin die Schmiermittelölzusammensetzung eine Basenzahl, gemessen durch das Perchlorsäureverfahren, von 15-125 mgKOH/g und eine kinematische Viskosität bei 100°C von 10-30 mm²/s hat und
worin die Schmiermittelölzusammensetzung als Komponente (A) enthält:
(A1) ein Ca-Phenat-Reinigungsmittel und
(A2) ein anderes metallisches Reinigungsmittel als irgendein Ca-Phenat-Reinigungsmittel,
wobei die Schmiermittelölzusammensetzung wahlweise enthält:
(C-1') ein Succinimid mit zumindest einer Alkyl- oder Alkenylgruppe in einem Molekül davon oder einem borierten Derivat davon in einer Menge von nicht mehr als 0,015 Massen-%, ausgedrückt als Stickstoff, auf der Basis der Gesamtmasse der Zusammensetzung, und
worin ein Ph-Wert, dargestellt durch die folgende Formel, nicht mehr als 20 × 10⁻³ ist: $Ph - Wert = {C}_{Ca} \times 2 / \left({r}_{M}\times 40,08\right)$
worin in der Formel (1) C_{Ca} ein Calciumgehalt in Massen% ist, der von der Komponente (A1) stammt, und r_{M} ein Metallverhältnis der Komponente (A1) ist und
worin das Metallverhältnis der Komponente (A1) durch die folgende Formel (2) berechnet ist: $\begin{matrix}Metallverhältnis der Komponente \left(A1\right) = Calciumgehalt in \\ Massen - % im Ca-Phenat-Reinigungsmittel , das die \\ Komponente \left(A1\right) ist/Calciumgehalt in Massen - % , der von \\ der Seifenbase im Ca-Phenat-Reinigungsmittel stammt , das \\ die Komponente \left(A1\right) ist\end{matrix}$

2. Zylinder-Schmiermittelölzusammensetzung für einen Kreuzkopfdieselmotor, ausgerüstet mit dem Gaswäscher nach Anspruch 1, worin die Schmiermittelölzusammensetzung die Komponente (C-1') in einer Menge von größer als 0 Massen-% und nicht mehr als 0,015 Massen-%, ausgedrückt als Stickstoff auf der Basis der Gesamtmasse der Zusammensetzung enthält.

3. Zylinder-Schmiermittelölzusammensetzung für einen Kreuzkopfdieselmotor, ausgerüstet mit dem Gaswäscher nach Anspruch 1 oder 2, worin die Komponente (A2) ein Ca-Sulfonat und/oder ein Ca-Salicylat ist.

4. Verfahren zum Schmieren eines Zylinders eines Kreuzkopfdieselmotors, ausgerüstet mit einem Gaswäscher, enthaltend:
Betreiben des Kreuzkopfdieselmotors, während die Schmiermittelölzusammensetzung nach einem der Ansprüche 1 bis 3 zum Zylinder des Kreuzkopfdieselmotors, der mit dem Gaswäscher ausgerüstet ist, geführt wird und
Reinigen von zumindest einem Teil des Gases, das von dem Zylinder im Gaswäscher abgelassen wird.

5. Verfahren zum Schmieren des Zylinders des Kreuzkopfdieselmotors, ausgerüstet mit einem Gaswäscher, nach Anspruch 4, worin das Reinigen in dem Gaswäscher das Kontaktieren des Gases, das in den Gaswäscher eingeführt ist, mit Wasser und/oder einer basischen wässrigen Lösung enthält.

6. Zylinder-Schmiermittelölzusammensetzung für einen Kreuzkopfdieselmotor, ausgerüstet mit einem Gaswäscher, enthaltend:
ein Grundöl und
(A) ein metallisches Reinigungsmittel und
(B) einen Demulgator in einer Menge von 0,02-5,0 Massen% auf der Basis der Gesamtmasse der Zusammensetzung, worin die Komponente (B) eine oder mehrere Polyetherverbindungen ist,
worin die Schmiermittelölzusammensetzung wahlweise enthält:
(C) ein stickstoffhaltiges ascheloses Dispergiermittel in einer Menge von nicht mehr als 0,2 Massen-%, ausgedrückt als Stickstoff, auf der Basis der Gesamtmasse der Zusammensetzung,
worin die Schmiermittelölzusammensetzung eine Basenzahl, gemessen durch das Perchlorsäureverfahren, von 15-125 mgKOH/g und eine kinematische Viskosität bei 100°C von 10-30 mm²/s hat.

7. Zylinder-Schmiermittelölzusammensetzung für den Kreuzkopfdieselmotor, ausgerüstet mit dem Gaswäscher, nach Anspruch 6, worin die Schmiermittelölzusammensetzung wahlweise enthält:
(C) das stickstoffhaltige aschelose Dispergiermittel in einer Menge von nicht mehr als 0,12 Massen-%, ausgedrückt als Stickstoff, auf der Basis der Gesamtmasse der Zusammensetzung.

8. Zylinder-Schmiermittelölzusammensetzung für den Kreuzkopfdieselmotor, ausgerüstet mit dem Gaswäscher, nach Anspruch 6 oder 7, worin die Schmiermittelölzusammensetzung (C) das stickstoffhaltige aschelose Dispergiermittel enthält.

9. Zylinder-Schmiermittelölzusammensetzung für den Kreuzkopfdieselmotor, ausgerüstet mit dem Gaswäscher, nach einem der Ansprüche 6 bis 8, worin ein Molekulargewicht im Zahlenmittel der Komponente (B) nicht weniger als 500 ist.

10. Zylinder-Schmiermittelölzusammensetzung für den Kreuzkopfdieselmotor, ausgerüstet mit dem Gaswäscher, nach einem der Ansprüche 6 bis 9, worin die Komponente (A) ein Ca-Phenat ist.

11. Verfahren zum Schmieren eines Zylinders eines Kreuzkopfdieselmotors, ausgerüstet mit einem Gaswäscher, enthaltend das Betreiben des Kreuzkopfdieselmotors, während die Schmiermittelölzusammensetzung nach einem der Ansprüche 6 bis 10 zum Zylinder des Kreuzkopfdieselmotors, der mit dem Gaswäscher ausgerüstet ist, geführt wird, und Reinigen von zumindest einem Teil des Gases, das von dem Zylinder im Gaswäscher abgelassen wird.

12. Verfahren zum Schmieren des Zylinders eines Kreuzkopfdieselmotors, ausgerüstet mit dem Gaswäscher, nach Anspruch 11, worin das Reinigen im Gaswäscher das Kontaktieren des Gases, das in den Gaswäscher eingeführt ist, mit Wasser und/oder einer basischen wässrigen Lösung enthält.

## Revendications

1. Composition d'huile de lubrification de cylindres pour un moteur diesel à crosse équipé d'un épurateur, comprenant :
une huile de base ; et
(A) un détergent métallique,
dans laquelle la composition d'huile de lubrification présente un indice de base mesuré par le procédé à l'acide perchlorique de 15 à 125 mg de KOH/g, et une viscosité cinématique à 100°C de 10 à 30 mm²/s ; et
dans laquelle la composition d'huile de lubrification comprend, en tant que composant (A),
(A1) un détergent phénate de Ca ; et
(A2) un détergent métallique autre qu'un quelconque détergent phénate de Ca ;
la composition d'huile de lubrification comprend optionnellement :
(C-1') un succinimide présentant au moins un groupe alkyle ou alcényle dans une molécule de celui-ci, ou un dérivé boré de celui-ci, en une quantité de pas plus de 0,015 % en masse en termes d'azote sur la base de la masse totale de la composition ; et
dans laquelle une valeur Ph représentée par la formule (1) suivante n'est pas supérieure à 20 × 10⁻³ : $valeur Ph = {C}_{Ca} \times 2 / \left({r}_{M}\times 40,08\right)$
dans laquelle dans la formule (1), C_{Ca} représente la teneur en calcium en % en masse issue du composant (A1), et r_{M} représente un rapport métallique du composant (A1) ; et
dans laquelle le rapport métallique du composant (A1) est calculé par la formule (2) suivante : $\begin{matrix}rapport métallique du composant \left(A1\right) = teneur en calcium en % en masse dans le \\ détergent phénate de Ca qui est le composant \left(A1\right) / teneur en calcium en % en masse \\ issue d ′ une base de savon dans le détergent phénate de Ca qui est le composant \left(A1\right)\end{matrix}$

2. Composition d'huile de lubrification de cylindres pour le moteur diesel à crosse équipé de l'épurateur selon la revendication 1,
dans laquelle la composition d'huile de lubrification comprend le composant (C-1') en une quantité supérieure à 0 % en masse et non supérieure à 0,015 % en masse en termes d'azote sur la base de la masse totale de la composition.

3. Composition d'huile de lubrification de cylindres pour le moteur diesel à crosse équipé de l'épurateur selon la revendication 1 ou 2,
dans laquelle le composant (A2) est un sulfonate de Ca et/ou un salicylate de Ca.

4. Procédé de lubrification d'un cylindre d'un moteur diesel à crosse équipé d'un épurateur, comprenant :
le fonctionnement du moteur diesel à crosse tout en fournissant la composition d'huile de lubrification selon l'une quelconque des revendications 1 à 3 au cylindre du moteur diesel à crosse équipé de l'épurateur ; et
la purification d'au moins une partie du gaz évacué à partir du cylindre dans l'épurateur.

5. Procédé de lubrification du cylindre du moteur diesel à crosse équipé de l'épurateur selon la revendication 4,
dans lequel la purification dans l'épurateur comprend la mise en contact du gaz introduit dans l'épurateur avec de l'eau et/ou une solution aqueuse basique.

6. Composition d'huile de lubrification de cylindres pour un moteur diesel à crosse équipé d'un épurateur, comprenant :
une huile de base ;
(A) un détergent métallique, et
(B) un désémulsifiant en une quantité de 0,02 à 5,0 % en masse sur la base de la masse totale de la composition, dans laquelle le composant (B) est un ou plusieurs composés polyéther.
dans laquelle la composition d'huile de lubrification comprend optionnellement :
(C) un dispersant sans cendres contenant de l'azote en une quantité de pas plus de 0,2 % en masse en termes d'azote sur la base de la masse totale de la composition,
dans laquelle la composition d'huile de lubrification présente un indice de base mesuré par le procédé à l'acide perchlorique de 15 à 125 mg de KOH/g, et une viscosité cinématique à 100 °C de 10 à 30 mm²/s.

7. Composition d'huile de lubrification de cylindres pour le moteur diesel à crosse équipé de l'épurateur selon la revendication 6,
dans laquelle la composition d'huile de lubrification comprend optionnellement :
(C) le dispersant sans cendres contenant de l'azote en une quantité de pas plus de 0,12 % en masse en termes d'azote sur la base de la masse totale de la composition.

8. Composition d'huile de lubrification de cylindres pour le moteur diesel à crosse équipé de l'épurateur selon la revendication 6 ou 7,
dans laquelle la composition d'huile de lubrification comprend :
(C) le dispersant sans cendres contenant de l'azote.

9. Composition d'huile de lubrification de cylindres pour le moteur diesel à crosse équipé de l'épurateur selon l'une quelconque des revendications 6 à 8,
dans laquelle un poids moléculaire moyen en nombre du composant (B) n'est pas inférieur à 500.

10. Composition d'huile de lubrification de cylindres pour le moteur diesel à crosse équipé de l'épurateur selon l'une quelconque des revendications 6 à 9,
dans laquelle le composant (A) est un phénate de Ca.

11. Procédé de lubrification d'un cylindre d'un moteur diesel à crosse équipé d'un épurateur, comprenant :
le fonctionnement du moteur diesel à crosse tout en fournissant la composition d'huile de lubrification selon l'une quelconque des revendications 6 à 10 au cylindre du moteur diesel à crosse équipé de l'épurateur ; et
la purification d'au moins une partie du gaz évacué à partir du cylindre dans l'épurateur.

12. Procédé de lubrification du cylindre du moteur diesel à crosse équipé de l'épurateur selon la revendication 11,
dans lequel la purification dans l'épurateur comprend la mise en contact du gaz introduit dans l'épurateur avec de l'eau et/ou une solution aqueuse basique.
